

# UNITED STATES PATENT OFFICE.

JOHN J. MCINTYRE, OF INVERNESS, NOVA SCOTIA, CANADA.

## PROCESS OF TREATING WOOD TO BE USED IN MAKING PLUNGERS, &c.

1,194,404.

Specification of Letters Patent. Patented Aug. 15, 1916.

No Drawing.

Application filed October 13, 1914. Serial No. 866,527.

To all whom it may concern:

Be it known that I, JOHN J. MCINTYRE, a subject of the King of Great Britain, residing at Inverness, in the Province of Nova Scotia and Dominion of Canada, have invented certain new and useful Improvements in Processes of Treating Wood to Be Used in Making Plungers, &c., of which the following is a specification.

10 This invention relates to mine pumps and has special reference to the production of efficient material for manufacturing plungers, valve seats and valves to be used in said pumps.

15 Another object of this invention is the production of a simple and efficient process for treating or preparing the wood used in making plungers, valve seats and valves which are used in connection with mine pumps.

20 Other objects and advantages of the present invention will appear throughout the following specification and claims.

By actual experience I have found that the action of water upon metal out of which the plungers, valve seats and valves are usually made in mining pumps, causes the metal to be severely attacked due to the acid contained in the water, and thereby causes the metal to readily deteriorate, and hence, make it necessary to replace those parts which have become worn or otherwise unfit for use. In fact, I have found by experience that the destruction of these metal parts of the pump has been so rapid as to make it necessary to 30 replace the same several times every second or third week where the pump is used constantly, thereby causing considerable loss and inconvenience to the operator of the pump. For the above reason I have experimented 35 with the use of different materials out of which these several portions of the pump may be manufactured, and found the following material and process would produce the desired result. I form the plungers, valve 40 seats, and valves of the ordinary construction, but in place of using metal I use hard wood specially treated and seasoned. It is preferable to use rock maple, beech or birch, and I first treat the wood as follows: I boil 45 the same in hard water for two hours and then boil the wood in linseed oil and pine tar for one hour, of the desired proportions or in a solution of alkaline salt; then while

the wood is still warm I coat the same with tallow and rub the tallow well into the wood 55 until the surface of the same is glossy. After the wood has been thus treated, the several parts are placed in their desired positions in the pump, and the pump may then be operated in the usual manner, and it will be 60 found that the plungers, valve seats and valves will last considerably longer and will give considerable more satisfaction than the usual metal employed in making these parts of the pump. It has been found by actual 65 experience that the placing of the wooden pieces within the pump will not only cause considerable saving in cost, but that these parts may be more easily placed within the pump and may obtain a better fit than the 70 metal parts which have been heretofore used.

It should be understood that the present invention especially relates to the method of using wooden plungers, valve seats, and valves in a pump, and in order to cause the 75 wood out of which the plungers, valve seats and valves are made to be of the best service in the pump, the wood is treated as above set forth.

Having thus described the invention what 80 is claimed as new, is:—

1. A pump of the class described having its plungers, valve seats and valves formed of hard wood which has been thoroughly boiled and treated with linseed oil and pine 85 tar, and afterward thoroughly coated and rubbed with tallow for the purpose of producing a glossy surface and making the same water-proof.

2. A method for preparing valve seats, 90 plungers and valves for use in mining pumps which are formed of wood consisting in first boiling hard wood in water for two hours, then boiling the wood in linseed oil and pine tar of equal proportions for one hour, then 95 removing the hard wood from this liquid, then thoroughly coating the wooden parts with tallow and rubbing the same until the surface of the wooden parts is glossy.

In testimony whereof I hereunto affix my 100 signature in presence of two witnesses.

JOHN J. MCINTYRE.

Witnesses:

ANGUS McDOWELL,  
L. BAIN.